

Aug. 14, 1945.

H. FORD ET AL

2,382,047

MAGNESIUM

Filed Feb. 16, 1942



Fig. 1



Fig. 2

H. Ford  
E. E. Ensign  
A.C. Quinn  
INVENTOR.

Edwin C. McRae and  
Robert J. Dennis  
BY  
ATTORNEYS.

## UNITED STATES PATENT OFFICE

2,382,047

## MAGNESIUM

Henry Ford, Dearborn, Elbert Edwin Ensign, Ypsilanti, and Archibald C. Quinn, Dearborn, Mich., assignors to Ford Motor Company, Dearborn, Mich., a corporation of Delaware

Application February 16, 1942, Serial No. 431,078

13 Claims. (Cl. 75—67)

This invention relates to a process of producing metallic magnesium from the ores of that metal by dissociation under conditions of comparatively moderate temperature and high vacuum.

An object of this invention is the production of metallic magnesium directly in reguline form under controlled temperature and pressure as distinguished from the present commercial carbo-thermal reduction process in which the high temperatures of the electric arc are utilized at pressures of atmospheric or greater. Another object is to make possible the use of the common and readily available ores including magnesium carbonates, oxides and the dolomites. A further object of this invention is to form gases during the course of the reaction and in situ of the initial formation of magnesium to control the relative partial pressures obtaining in the system to obtain optimum magnesium production.

A feature of this invention is that it comprehends the dissociation of the magnesium-bearing material by heat alone rather than reduction by an intermediary reducing substance. As a corollary, the process increases the rate of dissociation at the desired temperatures, supplies gases at the points of dissociation to control the partial pressures, and combines the dissociated oxygen in forms which are essentially inert with the magnesium formed at the temperatures prevailing in the furnace or in the condensing chamber.

The reduction of magnesium oxides with carbon has been commercially practiced in the high temperatures prevailing in an electric arc. The difficulty with this procedure is that the pressures prevailing are atmospheric or greater; and, as at these pressures the reduction reaction is readily reversible, the magnesium vapor formed must be sharply quenched to the solid form to prevent reversion. The quenched magnesium is in the form of a pyrophoric powder which must be protected from contact with air. Certain disadvantages are encountered in this quenching, and further processing of the magnesium powder is required to reduce it to the reguline form.

The present invention avoids the difficulty in teaching a method of reducing the reversibility of the dissociation and its immediate product is metal in a crystalline or reguline form. It permits the operation to proceed at temperatures at which metallic containers may be used and the component substances placed under vacuum. It is, in essence, a one-step process which may be performed either by the batch method or continuously with apparatus within the scope of good engineering practice.

With these and other objects in view, the invention consists of the process and the steps thereof, described in this specification, claimed in the claims, and illustrated in the accompanying drawing in which:

Figure 1 is a diagrammatic representation of the dissociation reaction.

Figure 2 is a temperature-pressure chart showing the equilibrium conditions obtaining in the carbon-reduction of magnesium oxide.

Referring to Figure 1, the components are shown to be a magnesium bearing material, a source of the carbonate radical, and a quantity of carbon, all of these materials being intimately mixed in a finely divided state. Preferably all of them, but at least the carbonate, must pass a 200-mesh screen and are then formed in briquettes. The briquettes are placed in a closed metallic chamber which is heated while vacuum is applied until conditions of pressure below 3000 microns and of temperature in the range from 2000° to 2500° Fahrenheit are obtained. As a magnesium source, magnesium oxide (MgO), magnesium carbonate (MgCO<sub>3</sub>), dolomite (MgCO<sub>3</sub>—CaCO<sub>3</sub>), partially calcined dolomite (MgCO<sub>3</sub>—CaO), or calcined dolomite (MgO—CaO) may be used; but as it is essential that there be a source of the carbonate radical, if MgO or MgO—CaO be used, a carbonate must be added. Figure 1 indicates this source as "R" carbonate and it is to be understood that this may be either magnesium carbonate, calcium carbonate or any other economically feasible carbonate which dissociates when heated and whose resulting oxide does not flux at the temperatures obtaining.

If finely divided magnesium carbonate is used as the magnesium source, it decomposes, as explained later, only at relatively high temperatures to form magnesium oxide and carbon dioxide. On the other hand, if the source is originally magnesium oxide or magnesite, this primary decomposition is avoided. In any event there must be a finely divided carbonate which decomposes to form the appropriate oxide and the carbon dioxide. Therefore, as the heating continues, regardless of the original materials, the retort will contain solid magnesium oxide, nondecomposed carbonate, carbon dioxide, "R" oxide and carbon.

It may be shown that the magnesium oxide will dissociate without the intervention of any reducing or catalytic agent at the temperature and pressure now prevailing, but this dissociation proceeds at a very slow rate and unless the oxygen and magnesium are separably removed from the dissociation zone, reversal takes place. Even the

addition of carbon does not appreciably hasten this dissociation, although the oxygen, under such circumstances, unites with the carbon to form monoxide or dioxide as in the electric arc carbothermal process. Of course, higher temperatures reduce reversibility, but it must be remembered that it is very difficult to obtain retorts which will withstand the stresses when under vacuum at temperatures above 2100° F. Even Nichrome containers fail readily and the avoidance of even the smallest temperature increment is economically desirable as reflected in longer retort life.

At this point, reference is made to Figure 2, which shows the computed temperature-pressure equilibrium relations obtaining in the magnesium oxide and carbon reaction. It will be understood that specific values will differ when other materials are used and in the presence of other gases, but that the general conditions remain the same and the curves may be taken as indicative of these. Curve A shows the equilibrium condition as expressed in the partial pressure of magnesium vapor against temperature. It may be shown that the partial pressure of the CO must at least equal the vapor pressure of magnesium and accordingly curve B represents the permissive total pressure obtaining in the system for equilibrium condition were no other gases present. Therefore, as a general rule, at all points above curve B at least some magnesium will be dissociated and present as a gas.

To hasten dissociation and make the process economically feasible, it has been found that interface reactions must be encouraged between the solid components, the partial pressures controlled, and the dissociated oxygen removed from contact with magnesium vapor.

The magnesium oxide and the carbon remain solid through the temperature range and to maintain contact both must be present in a finely divided state. When either magnesium or calcium carbonate is very finely divided, a larger percentage of individually perfect crystals is found than when these materials are present in the massive form; and it has been established by Faraday that perfect crystals refuse to effloresce until the crystal face is fractured. Therefore, the dissociation does not proceed until the crystal is fractured by internal stress and that requires temperatures in the range of 2000° Fahrenheit, rather than approximately 1,600° Fahrenheit obtaining for the massive form. Therefore, the use of the finely divided carbonate insures that CO<sub>2</sub> will be released at approximately the temperature of MgO dissociation. The carbon dioxide when released will in turn substantially instantaneously react with the carbon forming a mixture of diluent gases comprising substantially carbon monoxide and a small amount of carbon dioxide. Hence the gases form currently with the release of magnesium vapors and remain in contact throughout.

Similar consideration is applied to the rate of magnesium oxide dissociation and it has been proved by Langmuir that the building up or breaking down of a solid phase occurs only at the interface between the two phases. (The works of Faraday and Langmuir may be found in a "Treatise of Physical Chemistry," by H. S. Taylor, second edition, volume 2, pages 1056 to 1069, inclusive.) Therefore, if merely the pure oxide and carbon be present, the dissociation occurs slowly, but if other foreign solid particles are added to provide interfaces, the rate of dissoci-

tion increases greatly. In the present process, the magnesium oxide engages in an interface reaction with the undecomposed magnesium carbonate or the calcium carbonate present. Thus, while magnesium carbonate alone is operable, if the oxide is used as a charge, another solid carbonate must be provided to obtain the desired interface reaction. The result of the interface reaction and the presence of the diluent is shown by curve C which indicates the actual temperature and pressure conditions at which dissociation will occur. This curve is below the others, and indicates that the dissociation is enhanced and the reversibility reduced under the stated conditions.

It will be noted from Figure 1 that on dissociation the chamber contains the gaseous magnesium and oxygen and removal of the latter is necessary. This is obtained by reaction with the carbon to form carbon monoxide or carbon dioxide which is much less reversible at the temperatures obtaining than oxygen, while the remainder of the oxygen forms an oxygen film on the carbon which is later released as the monoxide. The greater the amount which ultimately forms the monoxide, the lower will be the reversibility of the dissociation.

Much of the success of the process is due to the presence of the finely divided carbonates and the formation of the diluent carbon dioxide simultaneously in point of time and place with the dissociation of the magnesium oxide. Thus, as the oxide decomposes, carbon dioxide is immediately formed, which greatly reduces the effective partial pressure of the oxygen to a point where it is considerably less than one-half of the dissociation pressure of the magnesium oxide. This lessens the reversibility proportionately and permits operation of the process at correspondingly lower temperatures and higher pressures as indicated by curve C. Control of reversibility through the partial pressure has long been sought, but, to the applicants' knowledge, by the extraneous addition of inert gases of one form or another to the system. The formation of the desired diluent at the point of dissociation and as an essential element of the dissociation is novel, not only in reducing the partial pressures, but as an integral part of the entire dissociation process.

In operation, the retort is evacuated continuously to remove the gases formed. The portion containing the charge is heated to the high temperatures required, while adjacent the outlet, the wall temperature is maintained below the condensation point of magnesium vapor obtaining at that pressure. The vapor is then swept along by the evacuating gases until it reaches the cooler wall on which it condenses in crystalline form while the CO<sub>2</sub> and CO are disposed of through the vacuum pump. As a practical matter, a shallow charge is to be preferred as it is advisable to keep the path traversed by the gaseous magnesium through the charge at a minimum to discourage reversion.

Summing up the process, the novel essentials are that solid interfaces be provided to hasten dissociation and that diluent gases be formed at the same temperatures at which dissociation takes place. The former requires the presence of at least two solid components besides the magnesium oxide to be dissociated. The latter requires the presence of a very finely divided carbonate which will not decompose until substantially the dissociation temperature of the oxide is reached. Thus, both dissociation and reversibility are con-

trolled and the process brought within the range where suitable apparatus may be designed consonant with engineering practice.

The advantages include the relative cheapness of the prime material and the fact that the conversion is obtained at low temperatures without the use of an expensive reducing agent such as ferrosilicon, heretofore thought necessary. The process is safe, since no explosive or dangerous gases other than CO need be handled and the magnesium is in the crystalline form which is not pyrophoric. The problems of operation present little difficulty since both temperature and pressure are readily controlled and the process may be operated in batch pots or continuously by charging the retort through vacuum locks in a well-known manner.

We claim:

1. The process of producing reguline metallic magnesium comprising the steps of mixing a magnesium-bearing compound, carbon and a foreign finely divided crystalline component which remains solid at the temperature attained, briquetting such mixture, subjecting such briquettes to temperatures above 2100° Fahrenheit at an absolute pressure not to exceed 3000 microns, one of said materials decomposing to form carbon dioxide at said temperature and pressure, said carbon dioxide upon its release being converted substantially to carbon monoxide exhausting the gases formed therein and thereby flowing the magnesium vapors released to a cooler part of the system, and condensing said magnesium vapors under pressures and temperatures to obtain the metal in the solid, crystalline form.

2. The process of producing metallic magnesium from a mixture of finely divided magnesium-bearing compound, carbon, and a crystalline material decomposing to form carbon dioxide upon heating under pressures substantially below atmospheric, which includes the step of dissociating said magnesium-bearing compound and decomposing said source of carbon dioxide said carbon dioxide being converted almost simultaneously to carbon monoxide to reduce the partial pressure thereof.

3. The process of producing metallic magnesium which comprises the steps of heating a finely divided and intimate mixture of magnesium oxide, calcium carbonate, and carbon to temperatures from 2100° to 2500° Fahrenheit and at pressures not to exceed 1000 microns.

4. The process of producing metallic magnesium comprising the steps of heating a finely divided and intimate mixture of partially calcined dolomite and carbon to a temperature of between 2100° and 2500° Fahrenheit at an absolute pressure not to exceed 1000 microns.

5. The process of producing metallic magnesium comprising the steps of heating a finely divided and intimate mixture of magnesium carbonate, calcium carbonate and carbon at temperatures from 2100° to 2500° Fahrenheit at an absolute pressure not to exceed 1000 microns.

6. In the process of producing metallic magnesium from the ores thereof, the step of providing an inert diluent gas evolved from the crystalline substance of the charge substantially simultaneously with the production of the gaseous magnesium and intimately mixed therewith said reactions occurring at a temperature of 2100°-2500° F. and at an absolute pressure not to exceed 1000 microns.

7. In the process of producing metallic magnesium from the ores thereof, the step of provid-

ing a diluent gas substantially simultaneously with the production of the gaseous magnesium, said diluent gas being formed by thermal decomposition of a crystalline carbonaceous substance contained in the charge at substantially the same temperature at which the vaporous magnesium is formed of a solid substance intimately mixed with said ore said reactions occurring at a temperature of 2100°-2500° F. and at an absolute pressure not to exceed 1000 microns.

8. In the process of producing metallic magnesium from the reaction of the carbon and the ores thereof, the step of providing diluent gases resulting from the reaction of carbon dioxide gas and said carbon substantially simultaneously with the production of the gaseous magnesium, said diluent being formed by thermal decomposition of a carbonate at substantially the same temperature at which the vaporous magnesium is formed, said carbonate being intimately mixed with said ore said reactions occurring at a temperature of 2100°-2500° F. and at an absolute pressure not to exceed 1000 microns.

9. In the process of producing metallic magnesium from the reaction of carbon and the ores thereof, the step of providing diluent gases resulting from the reaction of carbon dioxide and a portion of said carbon substantially simultaneously with the production of the vaporous magnesium, said diluent being formed by the thermal decomposition of a carbonate at substantially the same temperature at which the vaporous magnesium is formed, said carbonate being intimately mixed with said ore, the normal decomposition temperature of said carbonate being raised to substantially the magnesium formation temperature by reducing said carbonate to very small particles to increase the proportion of perfect crystals therein said reactions occurring at a temperature of 2100°-2500° F. and at an absolute pressure not to exceed 1000 microns.

10. The process of producing metallic magnesium from the ores thereof which comprises the steps of partially calcining dolomite to obtain a mixture consisting substantially of magnesium oxide and calcium carbonate, reducing the partially calcined material to a fine powder to increase the proportion of perfect carbonate crystals therein and thereby increase the temperature of decomposition of said carbonate, mixing finely divided carbon with said calcined material, forming briquettes of said mixture, placing said briquettes in a retort and applying heat and vacuum thereto, said temperature being sufficient to dissociate said oxide and substantially simultaneously decomposing said carbonate, diluting the dissociated vaporous magnesium with the mixture of carbon monoxide and carbon dioxide formed from the carbonate and flowing the vaporous magnesium thereby from proximity of the briquettes, passing said vaporous magnesium while still under said reduced pressure over a cool surface to condense the magnesium in crystalline form, and removing said diluent from said system.

11. The process of producing metallic magnesium from the ores thereof which comprises the steps of finely dividing a carbonate, the oxide of which is characterized by remaining solid at the temperatures hereinafter attained in the system, said carbonate being divided sufficiently to increase the proportion of perfect crystals therein and the consequent temperature of decomposition thereof to at least 2000° F.,

intimately mixing magnesium oxide and carbon with said carbonate, forming said mixture into briquettes, placing said briquettes in a retort subjected to temperatures in excess of 2000° F. and absolute pressure below 3000 microns, decomposing said carbonate to form a solid oxide and carbon dioxide, said carbon dioxide reacting with said carbon forming a mixture of gases of substantially carbon monoxide and small amounts of carbon dioxide, dissociating said magnesium oxide to form vaporous magnesium, said magnesium and said mixture of gases being formed substantially simultaneously, flowing said vaporous magnesium from proximity of said briquettes by said mixture of gases, passing said vaporous magnesium while still subject to said reduced pressure over a cool surface to condense said magnesium to the solid crystalline state, and removing said diluent from said system.

12. A process for producing metallic magnesium which comprises the steps of heating magnesium bearing compound in the presence of finely divided carbon and finely divided foreign

5 crystalline substance capable of exerting a physical reaction with said magnesium bearing compound and at reaction temperature evolving an inert diluent gas stabilizing the equilibrium of vaporous magnesium and carbon monoxide to the right under an absolute pressure not to exceed 3000 microns.

10 13. A process for producing metallic magnesium from magnesium-bearing compound, comprising, steps of dissociating the magnesium compound by solid-solid interfacial reaction with a foreign crystalline agent, retarding the reassociation by a second interfacial reaction releasing a diluent gas which produces a vapor pressure of the magnesium at which it condenses without reassociation, and condensing the gaseous magnesium so formed, both said interfacial reactions occurring within the same range of temperature.

HENRY FORD.  
ELBERT EDWIN ENSIGN.  
ARCHIBALD C. QUINN.